

## UNITED STATES PATENT OFFICE

2,273,805

## PLATINUM ALLOY

Edmund Merriman Wise, Westfield, and Raymond Francis Vines, Garwood, N. J., assignors to The International Nickel Company, Inc., New York, N. Y., a corporation of Delaware

No Drawing. Application April 24, 1941, Serial No. 390,104. In Canada March 22, 1941

3 Claims. (Cl. 75—172)

The present invention relates to platinum alloys and more particularly to platinum alloys for use in jewelry, dental structures, and the like, and characterized by improved properties, especially hardness.

Heretofore, it has been proposed to incorporate iridium, ruthenium and/or osmium in platinum for use in jewelry, dental structures, electrical contacts, chemical equipment, etc., to harden the platinum. In addition to being more expensive than platinum, these alloys possessed certain disadvantages. The iridium-platinum alloys had a relatively higher melting point and were more difficult to cast in molds of the usual investments than was platinum. In addition, with the usual iridium contents of about 5% to 15%, the alloys were not very hard in the cast or fully annealed conditions and also had a higher density than platinum. The ruthenium-platinum and osmium-platinum alloys, especially those containing more than about 5% of ruthenium or osmium, gave off poisonous fumes during melting, had a higher melting point than platinum and did not have very good ductility.

Because of the disadvantages of the higher ruthenium and osmium content alloys, the art has been limited essentially to the iridium-platinum alloys for applications where increased hardness was required. However, as pointed out hereinbefore, the iridium-platinum alloys were costly, had a high melting point and were difficult to cast in the usual investments. The art has been constantly seeking to overcome these and other disadvantages and although many attempts were made to remedy the aforementioned shortcomings, none, as far as we are aware, was entirely successful when carried into practice commercially.

We have discovered that the prior art shortcomings can be avoided and that new and unexpected results can be obtained by using small controlled amounts of tin as a hardener in platinum and platinum base alloys. We have discovered that platinum-tin alloys possess improved hardnesses without loss of ductility, have lower melting points, and are easier to cast than the platinum-iridium alloys commonly used heretofore.

It is an object of the present invention to provide platinum-base alloys possessing improved hardnesses and containing small controlled amounts of tin.

It is another object of the present invention to provide a novel hard platinum alloy which has a lower melting point, is easier to cast, and is

lower in cost, while retaining good ductility, than the iridium-platinum alloy of similar hardness.

The present invention contemplates new hard platinum alloys for jewelry purposes, dental purposes, etc., which do not require the use of the rare and costly element iridium.

The invention also contemplates dental structures and jewelry and other articles of manufacture made of the alloys provided by the present invention.

Other objects and advantages of the invention will become apparent from the following description.

The invention provides improved platinum-base alloys containing small but effective amounts of tin, say about 0.35% to about 5%, and the balance substantially all platinum. In addition to tin and platinum, the alloys may contain small amounts less than about 5% of base metals, e. g., copper, nickel, molybdenum, tungsten, etc. The base metals may be present as minor constituents which improve certain other desired properties. Thus, the present invention includes platinum-copper-tin alloys containing tin and platinum in the amounts herein set forth and about 4% copper.

The tin-containing platinum alloys provided by the present invention do not contain over about 5% tin, preferably not more than 3% tin for best ductility. Tin contents in excess of about 5% appear to detrimentally affect the working properties and to cause cracking upon rolling, etc. Contrary to the belief that tin is detrimental in platinum and high platinum alloys due to its embrittling effect, we have made the astonishing discovery that platinum and high platinum alloys containing up to about 3% tin are ductile and exhibit satisfactory working properties. In general, it is preferred to maintain the tin content to

toward the minimum values, for example, about 0.5%, for alloys to be fabricated into intricate designs. A particularly suitable alloy for fabrication into intricate designs contains about 0.5% tin and the balance substantially all platinum.

A study of platinum alloys containing up to about 3% tin has revealed that such alloys apparently did not age harden and that the markedly increased hardness of the tin-containing alloys was not due to an age hardening effect. Some age hardening effects were observed in a 95/5 platinum-tin alloy.

The tin-containing platinum-base alloys of the present invention are characterized by improved hardnesses of at least about 80 Vickers hardness number.

The improved hardening effects of tin as contemplated herein are obtained in alloys containing a small but effective amount of tin, say about 0.35%, to about 5% tin, and the balance platinum, i. e., about 95% to 99.65% platinum. Preferably, the alloys contain at least about 0.45 or 0.5% tin and up to about 3% tin where maximum ductility is desired. We have found that small amounts of tin have much greater hardening effect than the same amount of known hardening agents for platinum such as iridium, ruthenium, osmium, rhodium, gold, silver, nickel, copper, iron, etc. The beneficial and improved effects of tin compared to iridium in platinum alloys are illustrated in Table I which sets forth the comparative hardnesses in the fully annealed condition and the approximate melting points of tin-platinum, and iridium-platinum alloys, as well as of substantially pure platinum.

Table I

| Alloy No. | Composition       | Melting Point | V. H. N. |
|-----------|-------------------|---------------|----------|
| 1.        | Pure platinum     | ° C.          |          |
|           | 5% Ir, 95% Pt     | 1,773         | 41       |
| 2.        | 10% Ir, 90% Pt    | 1,800         | 75       |
| 3.        | 15% Ir, 85% Pt    | 1,850         | 110      |
| 4.        | 5% Pd, 95% Pt     | 1,910         | 143      |
| 5.        | 0.5% Sn, 99.5% Pt | 1,750         | 60       |
| 6.        | 3.0% Sn, 97% Pt   | 1,740         | 81       |
| 7.        | 5.0% Sn, 95% Pt   | 1,620         | 160      |
|           |                   | 1,430         | 210      |

V. H. N. = Vickers hardness number (10 kg. load) after 50% cold reduction followed by annealing at 1,100° C. for 30 minutes and water quenching.

Alloys Nos. 5, 6 and 7 which were made in accordance with the present invention show marked increases in hardness, while retaining good ductility with comparatively small amounts of tin. Thus, alloy 5 which contained only about 0.5% tin, balance platinum, had a higher hardness than a tin-free platinum alloy containing 5% of the hardening element iridium, as illustrated by alloy No. 1. Furthermore, alloy No. 5 which is made in accordance with the present invention costs considerably less than prior art alloy No. 1. Based on current prices alloy No. 5 costs about \$5.65 less per ounce than does alloy No. 1. Alloys No. 6 and No. 7 which contained about 3% and about 5% tin, respectively, possessed higher hardnesses than alloys No. 2 and No. 3 which contained 10% and 15% iridium, respectively. The accompanying beneficial effect of tin compared to iridium in lowering the melting point while increasing the hardness is clearly illustrated in Table I.

In addition to platinum and tin, the alloys of the present invention may contain small amounts of incidental or minor constituents and impurities and when we state that platinum constitutes the "balance" or that the "balance" is substantially all platinum we do not intend to exclude small amounts of incidental or minor constituents and impurities. Thus, the alloys may contain small amounts of base metals, for example, copper, nickel, molybdenum, tungsten, etc., in small amounts more than 0.01% and less than 5%. Likewise, the platinum-base alloys may contain small amounts of other known non-platinum group metal hardeners of platinum to supplement the beneficial effects of tin. Furthermore, the alloys may contain small amounts of iron, magnesium, calcium and other elements com-

monly associated with platinum and platinum alloys. The platinum used in making the alloys of the present invention may contain small amounts of one or more platinum group metals other than platinum. It is known that platinum available in commerce sometimes contains small amounts of other platinum group metals carried over from the ore, incorporated during processing, etc. Some of the purer grades of commercially available platinum may contain only about 0.001% or 0.01% of other platinum group metals while less pure grades may contain more. As will be apparent to those skilled in the art, the incidental elements and impurities contained in platinum may be carried over into the final alloy or article. It is to be understood that when it is stated that the balance is "platinum" or "substantially all platinum," we do not exclude from the scope of the expression incidental and minor constituents and impurities which may be present in such amounts as occur in commercially available platinum and in commercially produced platinum products, or in amounts not adversely affecting the desired properties of the platinum-base alloy.

The present invention provides hard articles of manufacture made of the platinum alloys described hereinbefore and containing small but effective amounts of tin, for example, alloys containing about 0.35% to about 5% tin and the balance substantially all platinum, said platinum alloys possessing improved castability when molten and improved hardness in the solid state while retaining good ductility. The articles contemplated herein may be made of cast or wrought alloys. An illustrative example of a suitable wrought alloy for the manufacture of articles where high platinum group metal content and good workability combined with adequate hardness is required contains 0.5% tin and balance substantially all platinum. Larger amounts of tin may be used where high purity is not a primary factor but where good ductility is desired it is preferred that the tin content not exceed about 3%. An illustrative example of a cast alloy and casting suitable for articles where high hardness combined with adequate ductility are primary factors and where highest purity is not essential contains 1% to 3% tin and the balance substantially all platinum.

Illustrative examples of wrought and/or cast articles within the scope of the present invention include cast and wrought dental structures, restorations and the like, for example, cast dental restorations, such as, bridges, inlays, crowns, abutments, etc.; cast and wrought jewelry, for example rings, chains, brooches, clips, pins, enamelled jewelry, etc., especially when such items are mounted with diamonds. High hardness is desirable to insure retention of gems, to prevent distortion and to reduce scratching and wear. The corrosion-resisting properties, refractory properties, etc., combined with improved hardness and wear resistance render the alloys of the present invention also suitable for use in such articles as chemical ware and equipment, electric contacts, etc.

Although the present invention has been described in conjunction with preferred embodiments, it is to be understood that modifications and variations may be resorted to without departing from the spirit and scope of the invention, as those skilled in the art will readily understand. Such variations and modifications apparent to those skilled in the art are considered

to be within the purview and scope of the appended claims.

We claim:

1. A platinum alloy comprising a small but effective amount up to about 5% of tin and the balance substantially all platinum.

2. A workable platinum alloy comprising about

0.35% to about 3% tin and the balance substantially all platinum.

3. A workable platinum alloy comprising about 0.5% tin and the balance substantially all platinum.

EDMUND MERRIMAN WISE.  
RAYMOND FRANCIS VINES.